

July 4, 1950

A. E. CALKINS ET AL.

2,514,311

PROCESS OF MANUFACTURING AN ALUMINUM BASE GREASE

Filed Dec. 8, 1948



Austin E. Calkins  
Ralph Darley  
Alan Beerbower  
Inventors

By *John M. Thomas* Attorney

Patented July 4, 1950  
2,514,311  
A process for the manufacture of aluminum base greases, comprising the steps of mixing a mineral base lubricating oil with an aluminum soap, adding thereto a crystallization modifier, and rapidly cooling the resulting mixture.

## UNITED STATES PATENT OFFICE

2,514,311

PROCESS OF MANUFACTURING AN  
ALUMINUM BASE GREASE

Austin E. Calkins, Westfield, N. J., and Ralph Darley, Glen Burnie, and Alan Beerbower, Baltimore, Md., assignors to Standard Oil Development Company, a corporation of Delaware

Application December 8, 1948, Serial No. 64,164

1 Claim. (Cl. 252—35)

1

The present invention relates to a process of preparing an aluminum base grease. It relates more particularly to an aluminum soap thickened lubricating grease prepared with mineral base lubricating oils so chosen and compounded that a stable grease of good texture and firm consistency is obtained and is capable of being produced by rapid continuous or semi-continuous processes.

In the prior art, a number of successful aluminum soap base greases have been prepared. Because of their smooth texture and other desirable properties, aluminum soap greases have come to be particularly favored for many uses, especially for the lubrication of chassis parts of automobiles, tractors, and the like. The prior art has recognized certain difficulties, however, in the preparation of aluminum soap greases. They pass through a peculiar transition stage in cooling from grease cooking temperature to normal temperature and a hard, grainy and very unsatisfactory structure is likely to result unless (1) the cooling is conducted very slowly with careful control, or (2) certain specific crystallization modifiers are employed to prevent the development of graininess, etc., during the transition from a rubbery structure to a smooth unctuous gel.

In the older prior art it was considered essential to cool aluminum soap greases very carefully, for example by running the molten grease into shallow pans where cooling was allowed to progress very slowly. This was a very slow and tedious process. More recently, as disclosed, for example, in the patent to Sproule and Zimmer, No. 2,394,567, and in the patent to Beerbower (one of the present inventors) and Zimmer, No. 2,449,580, it has been found that modern rapid production methods may be employed in making aluminum soap greases, provided crystallization modifiers such as alkylated mono-nuclear phenol or related materials such as resorcinol are used. Thus, in the Sproule and Zimmer patent, about 0.75% by weight of tertiary octyl phenol is added to an aluminum soap grease and such grease may then be prepared by mixing lubricating oil and aluminum soap at a temperature of about 280° to 300° F., and then running the hot mixture through a rapid chiller, e. g., a continuous close-clearance water-cooled chiller of the thin layer or scraped wall type. Similarly, a grease containing about

0.1 to 1% of resorcinol may be rapidly cooled as described in said Beerbower and Zimmer patent.

The patented processes and products just described are quite satisfactory, but the present invention is based upon the discovery that it is readily possible, by a choice of the particular types of mineral lubricating oil employed, to make aluminum soap greases which can be rapidly chilled and which have excellent texture and consistency in spite of such rapid chilling. Furthermore, this may be accomplished without using special additives as modifiers. The economics resulting from such a process are obvious and the product is found to be an excellent lubricating grease.

Specifically, we have found that by the proper choice and blending of appropriate types of mineral lubricating oil which are readily available, at least one of which contains as a natural ingredient a polar compound or group of compounds effective as suitable crystallization modifiers, a good aluminum soap grease may be prepared. The efficient continuous rapid cooling process may be used with such materials. A lubricating oil distillate which, without finishing, contains active crystallization modifying material comprising alkylated phenols, phenolic derivatives, naphthenic acids, etc., is commonly obtained in the simple distillation of Venezuelan or Coastal type crude oils. The quantity of such modifiers is commonly of the order of 1 to 1.5% by weight, in the lubricating oil distillate. This is more than is desired and more than is needed to modify the soap crystallization in the rapid or close-clearance cooling process, and greases prepared solely with this oil have very poor structures. Hence, according to this invention, it is necessary to dilute the untreated distillate with a sufficient quantity of refined or neutral oil which has been treated (acid, clay, caustic, selective solvent, or the like) to reduce the free acid and phenolic content to very low values. The two oils are blended to obtain a stock having a modifier content which is about 0.1 to 1%, preferably 0.25 to 0.75% by weight, based on the finished grease. The optimum amount varies, depending upon the rapidity of cooling and intensity of mechanical working. By adjusting the proportions of unfinished distillate and neutral stock, the modifier

content may be accurately controlled within any reasonable desired limits.

While the exact composition of the modifier which is naturally present in crude naphthenic Venezuelan or Coastal oils is not fully known, it appears to be a mixture of polar compounds, phenols, organic acids, and acid-phenol substituted aromatics, all of which are soluble in potassium alcoholate or sodium hydroxide solution. These naturally occurring modifiers are effective to a very satisfactory degree for modifying the crystallization of aluminum soaps.

The extract from alkali treated oils may be used also by acidulating it. It contains modifiers of the same general type and may, under some circumstances, be an economical process.

In the drawing, there is shown a flow diagram to illustrate the simplicity and obvious advantages of the process more clearly. As shown therein, the Venezuelan or other naphthenic crude oil is subjected to ordinary vacuum distillation to separate the lighter fuel distillate and the heavier asphalt from the intermediate lubricating oil distillate. The lubricating oil distillate is then separated into two streams so that part of it goes to the grease cooking unit while another part is subjected to normal finishing operations. If desired, lubricating oil distillate from other operations may be brought into the normal finishing stage for acid treatment, soda washing, re-distillation over sodium hydroxide, and the like, as indicated above.

The finished neutral stock is then taken to the cooker where it is blended, in suitable proportions depending on the desired modifier content, with the unfinished distillate, and also the aluminum stearate or other aluminum soap. Aluminum stearate is specifically preferred, but other aluminum soaps of fatty acids of 12 to 22 carbon atoms such as hydrogenated fish oil acids, for example, may be used. The saturated fatty acids of this range are preferred because of their superior stability against oxidation. The proportions of finished and unfinished oils will usually be from about 1 to 4 parts by weight of finished or neutral stock combined with 10 to 2 parts by weight of the raw or unfinished oil. The aluminum soap content, based on the weight of the finished grease, is within the limits of about 3% to 30%, a range of 5 to 15% being generally preferred.

As the ingredients are mixed, they are heated to a temperature of at least 250° F. and may be heated as high as 350° F. The heating need not be long continued. In the continuous process, for example, heating is only momentary, i. e., long enough for the ingredients to attain the temperature of 250° F. to 350° F., with complete solvation, and the heated mixture is then passed in continuous flow to the rapid cooler.

The rapid cooler, which may be of the close clearance type, water jacketed, with or without scrapers, or a close fitting worm impeller, is arranged to bring the temperature down below the normal transition temperature range of about 70° to 160° F., for example to a temperature of between 70° and 100° F. From the cooler, the product may be packaged directly inasmuch as the final setting up and crystallization of the soap structure, which forms the body or framework of the gel, takes place very satisfactorily in the final package.

Although the flow plan just described suggests using oil which by-passes the finishing operation along with oil which goes through the finishing

operation, it will be self-evident that the finished stock may be any substantially neutral oil, derived from naphthenic or Coastal crude, or a Pennsylvania type oil. The latter, which is substantially neutral when removed from the still, commonly will require no finishing treatment. The product of the invention thus may comprise various types of neutral or substantially neutral stock combined with the unfinished naphthenic oil.

#### Example

As an example of the operation of this invention, the following may be cited: An unfinished Venezuelan distillate (from Lagunillas crude) and a finished Coastal distillate were selected as the two oil components. These oils had the following characteristics:

|                                 | Untreated Venezuelan Distillate | Finished Coastal Lubricating Oil |
|---------------------------------|---------------------------------|----------------------------------|
| Viscosity at 100° F. (SSU)      | 1214                            | 916                              |
| Viscosity at 210° F. (SSU)      | 78.4                            | 70.5                             |
| Gravity (API)                   | 18.2                            | 23.1                             |
| Flash Point, °F. (Open Cup)     | 445                             | 450                              |
| Pour Point, °F. (ASTM)          | +5                              | 0                                |
| Saponification No.              | 2.1                             | 0.14                             |
| Color (Tag-Robinson)            | Below 1                         | 10½                              |
| Cast (Color by reflected light) | Blue-Green                      | Blue                             |

These oils were then mixed with a commercial aluminum stearate in the following proportions:

| Ingredient:           | Per cent by weight |
|-----------------------|--------------------|
| Aluminum stearate     | 6.00               |
| Venezuelan distillate | 62.30              |
| Finished Coastal oil  | 31.70              |

These ingredients were stirred together at 90° F. in a conventional grease kettle, and heated to a temperature of 310° F. The resulting hot fluid mixture was then cooled continuously in a scraped surface cooler (known commercially as a "Votator") to below its transition range, preferably below 100° F., for example 92° F. During a 24 hour standing period, the product gelled to a firm grease having the following characteristics:

|                                                                   |                  |
|-------------------------------------------------------------------|------------------|
| Unworked penetration (ASTM)                                       | 214              |
| Worked penetration (ASTM)                                         | 326              |
| 1800 strokes worked penetration                                   | 327              |
| ASTM penetration after passage through a high pressure grease gun | 340              |
| Appearance                                                        | Semi-transparent |
| Oil separation (6 months at 77° F.)                               | None             |

The grease was subjected to all the conventional quality tests for pressure gun application, and was found to be very satisfactory.

It is obvious that the proportions of the treated and untreated oils may be varied and the quantities and types of soaps, or the fatty materials from which they are formed may be selected as desired. The conventional modifiers such as anti-oxidants, extreme pressure additives, tackiness agents, corrosion inhibitors, etc., may be employed if desired.

What is claimed is:

The process of preparing stable aluminum base lubricating greases of smooth texture which comprises combining about 62% by weight of unfinished Venezuelan distillate mineral oil of lubricating oil viscosity and containing about 1% to 1.5% by weight of polar compounds including phenols, naphthenic acids, and acid-phenol substituted aromatic compounds with about 32% of finished

Coastal oil as a diluent and about 6% of aluminum soap of substantially saturated fatty acids within the range of 12 to 22 carbon atoms as a thickener, heating the mixture to a temperature of above 300° F. and not higher than about 350° F., and thereafter rapidly cooling below about 100° F. in thin layers, accompanied by mechanical working.

AUSTIN E. CALKINS.

RALPH DARLEY.

ALAN BEERBOWER. 10

## REFERENCES CITED

The following references are of record in the file of this patent:

## UNITED STATES PATENTS

| Number    | Name             | Date          |
|-----------|------------------|---------------|
| 1,804,124 | Southard         | May 5, 1931   |
| 1,902,635 | Gebhardt         | Mar. 21, 1933 |
| 2,380,893 | Zimmer et al.    | July 31, 1945 |
| 2,431,453 | Beerbower et al. | Nov. 25, 1947 |